

July 31, 1945.

W. R. BREELER ET AL

2,380,821

POPPET VALVE AND VALVE SEAT FOR INTERNAL-COMBUSTION ENGINES

Filed Jan. 21, 1941



FIG. 1



FIG. 2



FIG. 3

ANALYSIS

C. 0.25% to 1.0%  
Mn. 4.0% to 8.5%  
Cr. 18.0% to 22.0%  
A total of elements selected  
from the group consisting  
of Mn. & Ni 5.0% to 8.5%

INVENTORS

Walter R. Breeler

Gurdon M. Butler Jr.

by 

ATTORNEY

## UNITED STATES PATENT OFFICE

2,380,821

POPPET VALVE AND VALVE SEAT FOR  
INTERNAL-COMBUSTION ENGINES

Walter R. Broeler and Gordon M. Butler, Jr.,  
Fredonia, N. Y., assignors to Allegheny Ludlum  
Steel Corporation, Pittsburgh, Pa., a corpora-  
tion of Pennsylvania

Application January 21, 1941, Serial No. 375,246

6 Claims. (Cl. 123—188)

Our invention relates to poppet valves and valve seats for internal combustion engines and particularly to alloy steels which are suitable for use in such valves and seats operating in engines using modern anti-knock fuels.

In the drawing, Fig. 1 is an elevation view of a poppet valve for an internal combustion engine; Fig. 2 is a plan view of a valve seat insert, drawn to a somewhat smaller scale than the valve in Fig. 1; and Fig. 3 is a section of Fig. 2 in the plane 3—3.

While the necessary and desirable physical characteristics of steels for use in engine valves and seats are well known, the problem of finding a steel embodying all of the necessary and most of the desirable properties is extremely difficult. Three important properties are high resistance to corrosion from the exhaust gases produced by modern fuels, high resistance to deformation at valve operating temperatures, and retention of a high degree of hardness after prolonged exposure to these temperatures.

Poppet valves, and particularly exhaust valves, are subjected to rapidly fluctuating stresses of great intensity while heated to elevated temperature by the gases resulting from the combustion of the fuel. Valves which are formed of steels having insufficient hot strength are subject, under these conditions, to gradual deformation. The heads are forced downwardly into the seat openings until they become concave or "dished" which changes the seat angle of the valve, prevents its closing tightly, and thus causes leakage, overheating and, eventually, failure.

In order finally to determine whether any steel will make a satisfactory valve the ultimate test, of course, requires that valves shall be made from the steel and run for prolonged periods in an internal combustion engine. The manufacturing and testing of valves in this way is a long and expensive procedure, and hence it is highly desirable to devise some preliminary test to which samples of steel can be easily put for the purpose of determining whether such steels warrant the expense of making and running valves made therefrom. The valve steel problem heretofore has been largely a "cut and try" problem, and therefore progress in developing new and better valve steels has been much slower than the extensively developed art of alloy steels would seem to warrant. It is well recognized however by the comparatively few workers in this highly specialized field of research that alloys which are highly resistant to hot oxidation and have high strength at elevated temperatures, as measured by ordi-

nary short-time, hot tensile tests, are not, *ipso facto*, suitable for internal combustion engine valves.

Accelerated tests which fairly indicate the probable corrosion resistance, in actual operation, of a valve made from steel of a given analysis were devised a few years ago but there has been no satisfactory test, so far as we are aware, by which the relative resistance of various steels to the "dishing" deformation above mentioned could be evaluated. In order preliminarily to determine this resistance we have devised a comparatively simple procedure in the form of a hot bend or "accelerated creep" test. According to our procedure, a short strip of the steel being studied is supported at its extremities in a furnace while a load is applied to the center thereof by means of a yoke connected to a rod carrying dead weights which hang below the furnace. At any given temperature a load can be chosen by successive trials so as to cause the strip to bend or deflect a predetermined amount in a specified time. By making, treating and testing all specimens exactly alike the relative resistances of the steels to the type of head deformation met in exhaust valves can be accurately determined, and, if the specimens are subjected to the test loads for 24 hours at 1400° F., this new testing method has been found to give a good indication of the relative resistances of steels to deformation in service, as determined by actual engine tests. Comparative experiments established that the usual, short-time, hot tensile test gives extremely unreliable indications as to the true value of steels for valve service. Many steels shown to be very strong by such tests but very weak by our "accelerated creep" test failed in actual engine tests.

In our tests, all specimens were rated according to the load in pounds required to cause a permanent bend or deflection of 0.020" therein when applied for 24 hours, and the numbers used hereinafter to indicate the resistance of the various steels to hot bending are to be understood as indicating such load in pounds. Thus we find that very weak steels may have ratings of less than 5. Most of the commercial ferritic valve steels will range from 10 to 15, and the best commercial austenitic valve steels will range from 20 to 30. No steels which we have subjected to this test have shown values much over 40.

The alloy steel from which our poppet valves are made contains the following essential alloying elements within the ranges stated; it being understood that the percentages used throughout

the specification and claims refer to percentages by weight.

|                                                                                | Per cent    |   |
|--------------------------------------------------------------------------------|-------------|---|
| Carbon                                                                         | 0.25-1.00   |   |
| Manganese                                                                      | 4.00-8.50   | 5 |
| Chromium                                                                       | 18.00-22.00 |   |
| A total of elements selected from the group consisting of manganese and nickel | 5.00-8.50   |   |
| Iron                                                                           | Balance 10  |   |

All specimens were hot worked from 17 lbs. ingots into strips and air-cooled after 30 minutes at 2000° F. The specimens were tested for Rockwell C hardness and magnetic saturation at 400 oersteds field strength, then heated at 1600° F. for 1 hour, air-cooled, reheated at 1400° F. for 1 hour, and retested. They were then subjected to the 24-hour "accelerated creep" or hot bend test and the hardness and magnetism again determined.

TABLE I

## Effect of varying chromium content

[C 0.5%, Mn 8%, Si 0.5%]

| Heat No. | Cr   | Mn  | Treatment (A), as air-cooled from 2,000° |           | Treatment (B), before test: 2,000° plus 1,600° plus 1,400° |           | Treatment (C), after test: (B) plus 1,400° 25 hrs.—air |           | Relative resistance to hot bending |
|----------|------|-----|------------------------------------------|-----------|------------------------------------------------------------|-----------|--------------------------------------------------------|-----------|------------------------------------|
|          |      |     | Rock-well                                | Mag. sat. | Rock-well                                                  | Mag. sat. | Rock-well                                              | Mag. sat. |                                    |
| P-213    | 17.9 | 7.8 | 34                                       | 100       | 37                                                         | 2,100     | 41                                                     | 6,200     | 39                                 |
| P-200    | 20.1 | 7.8 | 34                                       | 250       | 38                                                         | 2,100     | 39                                                     | 6,900     | 25                                 |
| P-85     | 22.0 | 7.8 | 29                                       | 1,450     | 33                                                         | 4,700     | 29                                                     | 5,300     | 12                                 |
| P-87     | 24.2 | 7.9 | 23                                       | 5,900     | 21                                                         | 5,900     | 22                                                     | 5,300     | 9                                  |
| P-107    | 26.1 | 7.8 | 18                                       | 9,000     | 18                                                         | 8,700     | 17                                                     | 8,300     | 8                                  |

Within these ranges the steel is wholly or nearly non-magnetic as rolled, or as quenched from about 2,000° F., but will become somewhat magnetic after reheating for more or less prolonged periods at temperatures of 1200° to 1400° F. In other words, the steel is neither wholly austenitic nor wholly ferritic but between these extremes.

We are aware that the prior art discloses a great

30 Here is apparent the combination of strength and hardness developed with chromium contents up to 20% with an abrupt drop in retained hardness and strength with chromium contents of 22% or more. The magnetic data indicate that in the 24 and 26% chrome alloys some of the so-called "sigma phase" is developing as the steels become less magnetic after reheating at the lower temperature.

TABLE II

## Effect of varying manganese content in a 20% chromium alloy

[0.5% C, 0.5% Si]

| Heat No. | Cr   | Mn   | Treatment (A), as air-cooled from 2,000° |           | Treatment (B), before test: 2,000° plus 1,600° plus 1,400° |           | Treatment (C), after test: (B) plus 1,400° 25 hrs.—air |           | Relative resistance to hot bending |
|----------|------|------|------------------------------------------|-----------|------------------------------------------------------------|-----------|--------------------------------------------------------|-----------|------------------------------------|
|          |      |      | Rock-well                                | Mag. sat. | Rock-well                                                  | Mag. sat. | Rock-well                                              | Mag. sat. |                                    |
| P-262    | 20.0 | 1.9  | 51                                       | 9,800     | 19                                                         | 15,200    | 15                                                     | 15,200    | 4                                  |
| P-264    | 20.0 | 3.6  | 41                                       | 1,800     | 27                                                         | 15,200    | 24                                                     | 14,200    | 7                                  |
| P-198    | 19.8 | 6.2  | 36                                       | 600       | 40                                                         | 12,000    | 38                                                     | 12,650    | 15                                 |
| P-200    | 20.1 | 7.8  | 24                                       | 250       | 38                                                         | 8,100     | 28                                                     | 6,900     | 25                                 |
| P-255    | 20.4 | 11.2 | 32                                       | 150       | 32                                                         | 200       | 20                                                     | 200       | 29                                 |
| P-256    | 20.4 | 12.9 | 28                                       | 50        | 27                                                         | 50        | 26                                                     | 150       | 22                                 |

deal of information about steels whose principal alloying ingredients are chromium and manganese but no one, so far as we are aware, has discovered the valuable characteristics possessed by steels containing these elements within the extremely narrow ranges above set forth when formed into poppet valves of internal combustion engines.

In the development of our steel a large number of experimental analyses was studied for the purpose of determining the particular ranges within which the various elements should be employed in order to attain the desired results and for the purpose of determining the effect of variations of the elements within these ranges. The results of our tests of a number of these steels are tabulated below.

60 These figures show that in the absence of nickel, the desired combination of strength and retained hardness is attained only in a very limited, upper portion of our total desired range (4 to 8.5% Mn).

The following table shows, however, that the addition of nickel makes possible a lower, wider, and more practical range of manganese, which is very important from a manufacturing standpoint.

70 Manganese and nickel are essentially complementary in our alloy; that is, when the manganese content is high, the nickel should be low, and vice versa. As the manganese approaches its upper limit, the nickel may be omitted altogether.

TABLE III

*Effect of 2% nickel in steels similar to  
in those Table II*

[20% Cr, 0.5% C, 0.3% Si, varying Mn]

| Heat No. | Cr   | Mn  | Ni  | Treatment (A) |           | Treatment (B) |           | Treatment (C) |           | Relative resistance to hot bending |
|----------|------|-----|-----|---------------|-----------|---------------|-----------|---------------|-----------|------------------------------------|
|          |      |     |     | Rock-well     | Mag. sat. | Rock-well     | Mag. sat. | Rock-well     | Mag. sat. |                                    |
| P-263... | 20.0 | 1.9 | 2.1 | 35            | 750       | 39            | 13,200    | 38            | 18,400    | 13                                 |
| P-196... | 19.7 | 4.1 | 2.0 | 38            | 600       | 39            | 10,800    | 37            | 12,100    | 19                                 |
| P-178... | 19.8 | 5.0 | 2.1 | 32            | 100       | 38            | 4,400     | 39            | 7,300     | 32                                 |
| P-179... | 19.9 | 5.9 | 2.1 | 30            | 50        | 33            | 1,600     | 35            | 4,400     | 31                                 |
| P-180... | 19.7 | 6.7 | 2.1 | 31            | 50        | 30            | 200       | 27            | 160       | 32                                 |
| P-201... | 20.0 | 7.7 | 2.0 | 29            | 50        | 29            | 100       | 28            | 150       | 30                                 |
| P-208... | 20.1 | 9.9 | 2.1 | 29            | 0         | 29            | 50        | 27            | 100       | 32                                 |

It is evident that 2% nickel makes the austenitic phase more stable and decreases the quantity of manganese required for the greatest strength and hardness. A desirable proportion would be 5-6% manganese with 1-2% nickel which gives almost the same properties as the 8% manganese steel without nickel.

20

corrosion by hot combustion products which characterizes our steels. The maintenance of this full contact area permits maximum flow of heat from the valve into the block or head, thus keeping the valve moderately cool and reducing corrosion to a minimum. Under the same conditions a weaker valve might deform by "dish-

TABLE IV

*Effect of adding nickel to a 20% chromium-6% manganese alloy*

[0.5% carbon, 0.3% silicon]

| Heat No. | Cr   | Mn  | Ni  | Treatment (A), as air-cooled from 2,000° |           | Treatment (B), before test: 2,000° plus 1,800° plus 1,400° |           | Treatment (C), after test: (B) plus 1,400° 25 hrs.—air |           | Relative resistance to hot bending |
|----------|------|-----|-----|------------------------------------------|-----------|------------------------------------------------------------|-----------|--------------------------------------------------------|-----------|------------------------------------|
|          |      |     |     | Rock-well                                | Mag. sat. | Rock-well                                                  | Mag. sat. | Rock-well                                              | Mag. sat. |                                    |
| P-198... | 19.8 | 6.2 | 0.0 | 36                                       | 600       | 40                                                         | 12,000    | 38                                                     | 12,650    | 16                                 |
| P-253... | 20.3 | 6.0 | 1.0 | 34                                       | 150       | 40                                                         | 5,000     | 40                                                     | 7,900     | 31                                 |
| P-179... | 19.9 | 5.9 | 2.0 | 30                                       | 50        | 33                                                         | 1,600     | 35                                                     | 4,400     | 31                                 |
| P-199... | 19.8 | 6.1 | 3.8 | 29                                       | 50        | 27                                                         | 50        | 27                                                     | 150       | 31                                 |

There is, evidently, no advantage in nickel contents which are higher than those needed to give the best strength, magnetic and hardness properties; but it will be noted that 1% nickel has made a great and valuable change in the character of the 6% manganese alloy. This steel appears to behave exactly like those containing 5% manganese and 2% nickel or the plain 8% manganese steels. In other words, small quantities of nickel when combined with manganese appear to be the equivalent of additional manganese in producing a steel having our desired properties.

The foregoing data reveal conclusively that there exists a narrow composition range within which steels may be made which are uniquely qualified to withstand the punishment borne by the exhaust valves of modern internal combustion engines. These steels develop a degree of hardness which is moderate but sufficient to withstand the wearing action on the valve stem and tip, and, moreover, this hardness is retained after heating to valve operating temperatures so that the seat portion of the head remains sufficiently hard to resist the indenting action of hard particles which may be trapped between the valve head and its seat. Our steels are strong at valve operating temperatures and will withstand the stresses developed in operation. Thus, the original contact area between the valve head and seat in the cool engine block or head of the motor is maintained. This last mentioned feature is an important factor in the superior resistance to

ing" down through the valve port, thus changing the seat angle and reducing the contact area. In such a case the valve overheats to such a degree that even the most corrosion-resistant materials fail.

Many investigators, heating chromium-manganese steels in air or oxygen, have found that they are more heavily scaled than chrome-nickel or plain chromium steels and have therefore concluded that they were unsuited for service at elevated temperatures. However, the corrosion of modern internal combustion engine valves is principally due not to oxygen but to the products resulting from the combustion of fuels. These products form a deposit on the valves which attacks the hot metal. Many tests have demonstrated that chromium-manganese steels, either with or without small quantities of nickel, are very resistant to such attack when the chromium content is not much below 20%. We have, therefore, fixed the lower chromium content of our alloy at about 18% because of the desirability of maintaining high resistance to such combustion products. The upper chromium limit, however, is sharply defined by the abrupt decrease in strength and hardness of those steels containing chromium in quantities above about 22%, as illustrated in Table I.

Steels with less than 4% manganese are soft, weak and predominantly ferritic, as shown in Tables II and III, while manganese in quantities

above about 8.5% reduces the hardness and does not increase the strength.

The maximum nickel content is not critical but is preferably not over 4%. As discussed in connection with Tables III and IV, a small quantity of nickel serves to effect a more than equal reduction in the manganese content, but too much nickel reduces the hardness to an undesirable degree. Thus, it may be said that our steel is essentially a chrome-manganese steel containing not less than 4% manganese with an optimum of from about 7% to 8.5% of this element. However, with manganese contents of less than this optimum, nickel, because of its greater effectiveness, weight for weight, in developing the desirable characteristic of our alloy, should also be used so that the total manganese plus nickel content is not less than about 5%.

The following table gives some indication of the effect of carbon:

TABLE V  
Effect of varying carbon in 20% Cr—6% Mn—2%  
Ni alloys  
[0.3% Si]

| Heat No.   | C    | Cr   | Mn  | Ni  | Treatment (A),<br>as air-cooled<br>from 2000° |              | Treatment (A),<br>before test:<br>2,000° plus<br>1,600° plus<br>1,400° | Treatment (C),<br>after test:<br>(B) plus 1,400°<br>25 hrs. air |              | Relative<br>resistance<br>to hot<br>bending |    |
|------------|------|------|-----|-----|-----------------------------------------------|--------------|------------------------------------------------------------------------|-----------------------------------------------------------------|--------------|---------------------------------------------|----|
|            |      |      |     |     | Rock-<br>well                                 | Mag.<br>sat. |                                                                        | Rock-<br>well                                                   | Mag.<br>sat. |                                             |    |
| P-248..... | .26  | 20.3 | 6.0 | 2.0 | 23                                            | 1,000        | 24                                                                     | 8,000                                                           | 26           | 3,600                                       | 34 |
| P-179..... | .54  | 19.9 | 5.9 | 2.0 | 30                                            | 50           | 33                                                                     | 1,600                                                           | 35           | 4,400                                       | 31 |
| P-251..... | 1.14 | 20.3 | 6.0 | 2.0 | 37                                            | 100          | 42                                                                     | 1,750                                                           | 44           | 3,400                                       | 19 |

The minimum carbon content is obviously fixed by the comparative softness of the low-carbon steels while the upper limit is indicated by the decrease in strength of those steels containing more than about 1% of carbon. In cases where high hardness is required, the upper portion of our carbon range will serve, but machining will be more difficult.

The tabulated data reveal that steels containing the essential elements of our invention in the optimum proportions are essentially non-magnetic as rolled or as rapidly cooled from 2000° F. but that they become at least moderately magnetic after prolonged reheating at about 1400° F., which constitutes one of the distinguishing features of our steel.

The word "valve" as used in the foregoing description and in the appended claims is to be understood as including in its meaning seat inserts for valves and other parts associated with valves and inserts which are subjected in use to contact with the exhaust gases of an internal combustion engine.

#### What we claim is:

1. An internal combustion engine valve formed of alloy steel characterized by being essentially non-magnetic as rolled, or when quenched from about 2000° F., but which becomes moderately magnetic after reheating at 1200° to 1400° F., in which condition it is highly resistant to deformation at elevated temperatures and retains high hardness after long heating at temperatures up to 1400° F.; said steel containing a plurality of elements of which the following within the ranges stated are then only elements necessary to attain said characteristics: from 0.25% to 1.0% of carbon, from 18% to 22% of chromium, from 5% to 8.5% selected from the group consisting of

manganese and nickel, and the balance iron; the total quantity of manganese in said steel being not less than 4% and not more than 8.5%.

2. An internal combustion engine valve formed of a readily forgeable alloy steel characterized by having a magnetic saturation value of less than about 1000 gauss as quenched from 2000° F., and from about 2000 to about 10,000 gauss after prolonged heating at 1400° F., said steel containing a plurality of elements of which the following within the ranges stated are the only elements necessary to attain said characteristics: from 0.25% to 1.0% of carbon, from 18% to 22% of chromium, from 5% to 8.5% selected from the group consisting of manganese and nickel, and the balance iron; the total quantity of manganese in said steel being not less than 4% and not more than 8.5%.

3. An internal combustion engine valve formed of an alloy steel characterized by being essentially

non-magnetic as rolled, or when quenched from about 2000° F., but which becomes moderately magnetic after reheating at 1200° to 1400° F., in which condition it is highly resistant to deformation at elevated temperatures and retains high hardness after long heating at temperatures up to 1400° F.; said steel containing a plurality of elements of which the following within the ranges stated are the only elements necessary to attain said characteristics: from 0.40% to 0.70% of carbon, from 19% to 21% of chromium, from 6% to 8.5% selected from the group consisting of manganese and nickel, and the balance iron; the total quantity of manganese in said steel being not less than 5% and not more than 8.5%.

4. An internal combustion engine valve formed of an alloy steel characterized by being essentially non-magnetic as rolled, or when quenched from about 2000° F., but which becomes moderately magnetic after reheating at 1200° to 1400° F., in which condition it is highly resistant to deformation at elevated temperatures and retains high hardness after long heating at temperatures up to 1400° F.; said steel containing a plurality of elements of which the following within the ranges stated are the only elements necessary to attain said characteristics: carbon 0.40% to 0.70%, chromium 18% to 22%, manganese 7.5% to 8.5%, and the balance iron.

5. An internal combustion engine valve formed of an alloy steel characterized by being essentially non-magnetic as rolled, or when quenched from about 2000° F., but which becomes moderately magnetic after reheating at 1200° to 1400° F., in which condition it is highly resistant to deformation at elevated temperatures and retains high hardness after long heating at temperatures up to 1400° F.; said steel containing a

plurality of elements of which the following within the ranges stated are the only elements necessary to attain said characteristics: carbon 0.40% to 0.70%, chromium 19% to 21%, manganese 5.5% to 7.5%, nickel 0.50% to 2.5%, nickel and manganese combined from 6% to 8.5%, and the balance iron.

6. An internal combustion engine valve formed of alloy steel characterized by being essentially non-magnetic as rolled, or when quenched from about 2000° F., but which becomes moderately magnetic after reheating at 1200° to 1400° F., in which condition it is highly resistant to defor-

mation at elevated temperatures and retains high hardness after long heating at temperatures up to 1400° F.; said steel containing a plurality of elements of which the following within the ranges stated are the only elements necessary to attain said characteristics: from 0.40% to 1.0% of carbon, from 18% to 22% of chromium, from 5% to 8.5% selected from the group consisting of manganese and nickel, and the balance iron; the total quantity of manganese in said steel being not less than 4% and not more than 8.5%.

WALTER R. BREELER.  
GURDON M. BUTLER, JR.

CERTIFICATE OF CORRECTION.

Patent No. 2,380,821.

July 31, 1945.

WALTER R. BREELER, ET AL.

It is hereby certified that error appears in the printed specification of the above numbered patent requiring correction as follows: Page 3, Table III, next to last column thereof, opposite "P-180", for the numeral "150" read --250--; page 4, Table V, seventh column thereof, in the heading, for "Treatment (A), before test:", read --Treatment (B), before test:--; line 69, claim 1, for the word "log" read --long--; line 72, same claim, for "then" read --the--; and that the said Letters Patent should be read with this correction therein that the same may conform to the record of the case in the Patent Office.

Signed and sealed this 29th day of January, A. D. 1946.

Leslie Frazer

(Seal)

First Assistant Commissioner of Patents.

plurality of elements of which the following within the ranges stated are the only elements necessary to attain said characteristics: carbon 0.40% to 0.70%, chromium 19% to 21%, manganese 5.5% to 7.5%, nickel 0.50% to 2.5%, nickel and manganese combined from 6% to 8.5%, and the balance iron.

6. An internal combustion engine valve formed of alloy steel characterized by being essentially non-magnetic as rolled, or when quenched from about 2000° F., but which becomes moderately magnetic after reheating at 1200° to 1400° F., in which condition it is highly resistant to defor-

mation at elevated temperatures and retains high hardness after long heating at temperatures up to 1400° F.; said steel containing a plurality of elements of which the following within the ranges stated are the only elements necessary to attain said characteristics: from 0.40% to 1.0% of carbon, from 18% to 22% of chromium, from 5% to 8.5% selected from the group consisting of manganese and nickel, and the balance iron; the total quantity of manganese in said steel being not less than 4% and not more than 8.5%.

WALTER R. BREELER.  
GURDON M. BUTLER, JR.

CERTIFICATE OF CORRECTION.

Patent No. 2,380,821.

July 31, 1945.

WALTER R. BREELER, ET AL.

It is hereby certified that error appears in the printed specification of the above numbered patent requiring correction as follows: Page 3, Table III, next to last column thereof, opposite "P-180", for the numeral "150" read --250--; page 4, Table V, seventh column thereof, in the heading, for "Treatment (A), before test:", read --Treatment (B), before test:--; line 69, claim 1, for the word "log" read --long--; line 72, same claim, for "then" read --the--; and that the said Letters Patent should be read with this correction therein that the same may conform to the record of the case in the Patent Office.

Signed and sealed this 29th day of January, A. D. 1946.

Leslie Frazer

(Seal)

First Assistant Commissioner of Patents.